

April 27, 1926.

1,582,718

F. WINKLER

MANUFACTURING ACTIVE CARBON

Filed Sept. 29, 1923



INVENTOR  
Fritz Winkler  
BY

Hausfeld Warland  
ATTORNEYS

Patented Apr. 27, 1926.

1,582,718

# UNITED STATES PATENT OFFICE.

FRITZ WINKLER, OF LUDWIGSHAFEN-ON-THE-RHINE, GERMANY, ASSIGNOR TO  
BADISCHE ANILIN- & SODA-FABRIK, OF LUDWIGSHAFEN-ON-THE-RHINE, GER-  
MANY, A CORPORATION OF GERMANY.

## MANUFACTURING ACTIVE CARBON.

Application filed September 29, 1923. Serial No. 665,627.

To all whom it may concern:

Be it known that I, FRITZ WINKLER, citizen  
of the German Empire, residing at Lud-  
wigshafen-on-the-Rhine, Germany, have in-  
5 vented new and useful Improvements in  
Manufacturing Active Carbon, of which the  
following is a specification.

My invention relates to a process enabling  
active carbon to be manufactured in an ordi-  
10 nary shaft furnace, thus avoiding the use  
of retorts heated from the outside, or of com-  
plicated revolving furnaces.

According to my invention a highly active  
15 carbon is obtained by applying direct heat,  
in a shaft furnace, to coal or other carbona-  
ceous material serving for the production of  
the active carbon, which may be coal, lignite,  
peat, earthy brown coal or wood or  
20 other material, whether or not prepared  
with alkalies or suitable salts and the like.  
This material in the form of a powder or in  
fine pieces is placed in the shaft furnace and  
hot combustion gases are introduced from  
25 below with sufficient pressure to make an  
agitation or a whirling motion of the coal  
or carbonaceous material within the said  
furnace. The material is thus thoroughly  
mixed and the whole mass is uniformly  
30 heated. Further the intimate contact with  
the hot fire gases causes the heating to take  
place very quickly; and a particularly effi-  
cient utilization of the heat can be obtained  
by using the gases issuing from the furnace  
35 for drying and preheating the material to be  
subjected to the activating treatment. The  
fire gases may also have an admixture of  
steam either continuously or periodically.  
The activated carbon can be readily with-  
40 drawn from the furnace by blowing it out  
from an opening near the bottom of the  
same by means of the fire gases.

In order to further illustrate the manner  
of carrying my invention into effect, I will  
45 describe it with reference to the accompany-  
ing diagrammatic drawing, but the inven-  
tion is in no way restricted to this example.  
Figure 1 represents a vertical section of a  
furnace embodying this invention.

A represents a combustion chamber in  
50 which fire gases are produced by burning  
fuel with air forced into the said chamber;  
preferably blue gas and air are used which  
are blown into the said chamber by means

of blower H in a tangential direction to  
make the combustion complete. The com-  
bustion gases then pass into a cylindrical  
shaft furnace B which is separated from the  
combustion chamber A by a plate of fire-  
clay, perforated with small apertures of  
say 5 millimetres width and carrying a layer  
55 of G of about 4 centimetres thickness of pieces  
of fireclay of hazelnut size. The furnace B,  
at its lower part, is conically reduced in size.  
The coal, for example peat charcoal, which  
is in grains of about 3 millimetres size is  
60 placed on the layer of the fireclay in a layer  
of about 40 centimetres in thickness. The  
fire gases are blown through this layer with  
a pressure of about 150 millimetres of water  
giving the peat coke on their passage a  
65 whirling movement. The coke is thus heat-  
ed very rapidly and after a few minutes is  
uniformly red-hot. When the temperature  
has reached about 800 degrees centigrade,  
steam is blown into the said combus-  
70 tion chamber A to mix there with the fire gases  
and the mixture is then allowed to act on  
the coke for about 10 minutes. The flue  
gases pass through the pipe J into the cham-  
ber E where fresh fuel is stored on a suit-  
75 able support L, for example a tipping grate,  
and after having preheated said charge of  
fuel they leave through waste pipe F. The  
material in furnace B after sufficient treat-  
80 ment is blown out through a discharge C  
into a chamber D, which chamber may be  
filled with an inert gas. This may be done  
by closing a waste pipe F and opening the  
discharge C which is connected by a pipe C<sub>1</sub>  
85 with a storage chamber D, from which the  
air has been removed and replaced by nitro-  
gen or carbon dioxide or other inert gas.  
When the furnace B is operated, the pipe C  
is closed by the stopper shown. By the  
90 closing of the waste pipe F the gases are  
compelled to escape through the said dis-  
charge C carrying along the active carbon  
that is ready into the chamber D where it is  
cooled. After opening the waste pipe F and  
95 closing the discharge opening C a fresh  
charge of peat coke is filled in from the  
chamber E and the furnace is ready for a  
further operation. In the chamber E a sup-  
100 ply of peat charcoal or other like material  
to be treated is kept and treated with the  
flue gas being dried and preheated thereby.  
105

The trap K is only opened when a fresh supply of fuel is charged into the furnace B.

It will be clear that no special means are necessary to prevent particles being blown right through C as in the chamber D the speed of the gases is reduced and the particles are allowed to settle.

The active carbon thus obtained is exceedingly active and may be used for example 10 for purifying gases from sulfuretted hydrogen by catalytic oxidation with air with very good result.

Instead of peat charcoal other carbonaceous or coal material such as for example 15 anthracite, lignite, lignite charcoal, or wood impregnated with potash or zinc chlorid or other salts, may be used and treated in the same manner yielding excellent results.

I claim:

20 1. The process of manufacturing active carbon which consists in treating carbonaceous material in a shaft furnace with hot combustion gases which are blown through the said material with sufficient pressure to establish a strong agitation of the material.

25 2. The process of manufacturing active carbon which consists in treating carbonaceous material impregnated with a salt promoting activation of coal in a shaft furnace

30 with hot combustion gases which are blown through the said material with sufficient

pressure to establish a strong agitation of the material.

3. The process of manufacturing active carbon which consists in treating lignite material in a shaft furnace with hot combustion gases which are blown through the said material with sufficient pressure to establish a strong agitation of the material. 35

4. The process of manufacturing active carbon which consists in treating lignite coke in a shaft furnace with hot combustion gases which are blown through the said material with sufficient pressure to establish a strong agitation of the material. 40

5. The process of manufacturing active carbon which consists in treating lignite coke in a shaft furnace with hot combustion gases and steam which are blown through the said material with sufficient pressure to 45 establish a strong agitation of the material. 50

6. The process of manufacturing active carbon which consists in treating lignite coke in a shaft furnace with hot combustion gases first alone then with an admixture of 55 steam, which are blown through the said material with sufficient pressure to establish a strong agitation of the material.

In testimony whereof I have hereunto set my hand.

FRITZ WINKLER.